

## 1

3,468,620

## PROCESS FOR THE DYEING OF POLYAMIDE FIBERS

Alfred Schaeuble, Richen, Ernst Adolf Räuchle, Basel, and Willi Leutenegger, Bottmingen, Basel-Land, Switzerland, assignors to J. R. Geigy A.G., Basel, Switzerland

No Drawing. Continuation-in-part of application Ser. No. 515,717, Dec. 22, 1965, which is a continuation-in-part of application Ser. No. 214,512, Aug. 3, 1962. This application Aug. 9, 1966, Ser. No. 571,194

Claims priority, application Switzerland, Aug. 11, 1961, 9,427/61, 9,428/61

Int. Cl. D06p 3/04

U.S. Cl. 8—54

49 Claims

## ABSTRACT OF THE DISCLOSURE

Polyamide fibers such as wool and nylon are dyed with a thickened acid dye composition containing the reaction product of a polyalkanolamine and a fatty acid, and a tetrahydronaphthalene sulfonic acid. Thioglycolic acid can be added to the dyeing mixture, which may also contain a "steam-blowing" control agent. The acid dye composition containing the dyeing composition used in the above process is also claimed herein.

This application is a continuation-in-part of copending patent application Ser. No. 515,717 filed Dec. 22, 1965 as a continuation-in-part of our patent application Ser. No. 214,512, filed Aug. 3, 1962 (forfeited in favor of the former). (Application Ser. No. 515,717 has been forfeited in favor of the present application.)

The present invention concerns a process for the dyeing of polyamide fibers and also the dye liquors suitable for this process.

The continuous dyeing of polyamide fibers is known. This is done by impregnating the polyamide material with an aqueous solution of acid wool dyestuffs which may be thickened, at temperatures under the drawing temperature of these dyestuffs, then after possibly drying the goods, steaming to fix the dyestuff and/or passing the goods through a hot acid bath ("acid shock process") and rinsing the goods so treated. As this process has disadvantages, e.g. it produces uneven dyeings, the addition of color carriers, to the impregnation liquors has already been suggested. The best of these have been found to be water-soluble condensation products of fatty acids having 8 to 14 carbon atoms or of mixtures of such acids with 2 equivalents of dialkanolamine. These condensation products are known as Kritchevsky bases and are described in U.S. Patent No. 2,089,212.

However, the use of these impregnation liquors has also a number of disadvantages. Above all, such impregnation liquors are not stable as after a few hours they separate irreversibly into two phases, one poor and the other rich in auxiliaries which makes level dyeing, particularly of large batches, more difficult. In addition, the ratio of each individual component to every other in the impregnation liquors must be exactly adjusted in order to obtain maximal dyeing yields. It is thus very difficult to obtain

## 2

uniform results by the known process. This adversely influences the industrial reliability of the process. In addition, if the dyestuff is to be fixed by passing the goods through a hot acid bath, an intermediate drying of the goods saturated with the impregnation liquor has been found to be necessary in order to avoid bleeding in the acid bath.

It has now surprisingly been found that polyamide fibers can be dyed by impregnating them with preferably thickened, aqueous solutions of acid wool dyestuffs at temperatures which are under the drawing temperature for these dyestuffs and the goods which have been impregnated and possibly dried can be finished by steaming and/or passing them through a hot acid bath, while avoiding all the disadvantages above mentioned, if the impregnation liquor contains, as color carrier, instead of the usual Kritchevsky bases as additives, a combination of:

(1) As color transfer agent, water soluble condensation product of 1 equivalent of fatty acid having 8 to 15 carbon atoms, or mixtures of such acids, and 1 to 3, preferably 2 equivalents of di- and/or trialkanolamine, or alkanol amides, and preferably di-lower alkanol amides of such acids, which are prepared as individual technical grade compounds;

(2) As anionic "steam-blowing" control agent.

(α) a preferably monosulfonated mono-alkyl-benzene or mono-alkyl-naphthalene wherein the alkyl moiety has from 8 to 20, and preferably from 9 to 14 carbon atoms, either in the form of the free monosulfonic acid or, preferably, of a water-soluble salt, especially an alkali metal or an ammonium salt thereof, the latter comprising in particular lower alkyl-ammonium and hydroxy-lower alkyl-ammonium salts;

(β) sulfonated  $\beta$ -tetrahydronaphthalene or a mixture of sulfonated  $\alpha$ - and  $\beta$ -tetrahydronaphthalenes, or such acid or acid mixture substituted by alkyl of 8 to 20, and preferably 9 to 14 carbon atoms, or the water-soluble salts thereof, preferably the salts of the same cations as under (α) and of the monosulfonic acids;

(γ) condensation products of formaldehyde, or glyoxal or acetaldehyde with, per mole thereof, about 1.2 to 2 moles of at least one, and preferably one or two of the following:

(i) benzene-sulfonic acid,  
(ii) naphthalene-sulfonic acid,  
(iii) tetrahydronaphthalene-sulfonic acid, and/or  
(iv) a methyl-substituted compound of (i) to (iii) inclusive, in free acid form or in the form of water-soluble salts thereof, preferably with the same cations as defined under (α); as well as

(3) If desired, thioglycolic acid or its water soluble salts which have a swelling action on polyamide.

The dyebaths thus prepared which are used as pad liquors, are preferably heated to about 40 to 60° C. before introducing the goods to be dyed thereinto. The pH of the pad liquors should be in the range of from 2 to about 8 to 9. Acid pH values are attained by addition of acidic substances, preferably formic or acetic acid to the pad liquors. When dyeing at pH values above 5.5 to 6, and particularly at the neutral to alkaline pH, it is often

recommended to treat the dyed fibers in a subsequent acid bath of a pH between 2 and 4.

In this way, uniform dyeings are obtained, even with large batches. In addition, a hot acid bath can be used without an intermediate drying and without any substantial bleeding.

The drawing temperature of the dyestuffs used, i.e. the temperature at which the dyestuff draws onto the fiber in about 1 minute, is generally 60° C. or higher. Thus in the process according to the invention, impregnation must be performed below this temperature.

This process is suitable for the continuous dyeing of polyamides, in particular, of wool. Principally  $\beta$ -tetrahydronaphthalene sulphonic acid or its water soluble salts are used according to the invention as component (2).

If, in order to obtain better penetration with the dyestuff used it is desired that the impregnation liquor also contain thioglycolic acid, the amount of the latter is preferably 0.1 to 3 g./liter.

The terms "tetrahydronaphthalene sulfonic acid," "sulfonated alkyl-benzene," "sulfonated tetrahydronaphthalene" and "disulfonated dinaphthyl-alkene" as used in this specification and the appended claims means the free acid as well as its water soluble, and particularly its alkali metal and ammonium salts, the latter comprising besides N-substituted ammonium also N-lower alkyl-substituted and N-(hydroxy-lower alkyl)-substituted ammonium salts.

While use of the control agents defined under (2)( $\beta$ ), supra, requires dyeing from a neutral to alkaline aqueous medium which is often undesirable, especially when dyeing wool, use of control agents as defined under (2)( $\alpha$ ) permits dyeing also from an acid medium and pH of which is at least 2 or higher. This makes it possible to use such industrially valuable dyes as Eriochrome Black T (C. I. No. 14645) which requires after-chroming at pH value below 5.

Particularly preferred are foam-forming control agents as defined under (2)( $\beta$ ), supra, which are alkyl-benzene-sulfonic acids or alkyl-phenol-sulfonic acids the alkyl moiety of which has from 9 to 14 carbon atoms, above all, 4-(1-methyl-undecyl)-benzene-sulfonic acid, 4-(tetrapropylene)-benzene-sulfonic acid or 4-nonyl-phenol-sulfonic acid, since these agents assist in obtaining particularly stable aqueous dye preparations and dyeings of even, deep shades.

These control agents are preferably used in the form of their water-soluble salts, especially their alkali metal or ammonium salts; however, their alkyl- or hydroxyl-alkyl-ammonium salts can also be used. Examples of suitable cations in such salts are the lithium, potassium, sodium, ammonium,  $\beta$ -hydroxy-ethyl-ammonium, or bis-( $\beta$ -hydroxymethyl)-ammonium ions.

The ratio of color transfer agent to "blowing" control agent should be in the range of from 1:1 to about 5:1.

The fatty acid di- and/or tri-alkanolamine condensation products used in the combination according to the invention can be produced according to the process described in U.S. Patent 2,089,212 mentioned above. Di- and tri-ethanolamine condensation products are preferred. They are produced by heating the fatty acids with 1-3 equivalents of di- and/or tri-ethanolamine, in particular diethanolamine, while splitting off more than 1 mol of water. Marketed mixtures known as coconut fatty acids are mainly used as fatty acids. They consist mainly of lauric acid and also contain in varying amounts the fatty acids having 8, 10 and 14 carbon atoms. The preferred diethanolamine can be wholly or partly replaced by other low alkanolamines, e.g. by triethanolamine, di-2-propanolamine or di-3-propanolamine. Particularly when using trialkanolamines and fatty acids having 8 to 12 carbon atoms, even in a molecular ratio of 1:1 with splitting off of 1 mol of water, the condensation product is sufficiently distributable in the dye liquor. Generally, however, it is advantageous if a multiple of the stoichiometric

amount, preferably double the amount of alkanolamine is used. In addition, it is favourable if at least one mol of the alkanolamine used also contains hydrogen bound to the nitrogen so that acid amide formation is possible. The condensation products used according to the invention are complex mixtures of fatty acid ethanolamides and fatty acid aminoalkanol esters. The fatty acid alkanolamide condensation products moiety is about 50-80% by weight and that of the esters is about 5-15% by weight. The difference mainly consists of uncondensed alkanolamine.

It is also possible to use, instead of such fatty acid amide/ester mixtures, products which consist of up to more than 90% of fatty acid amides which are obtained by reacting the esters of lower alkanols and higher fatty acids such as caprylic acid, pelargonic acid, capric acid, lauric acid, myristic acid, decyloxyacetic acid, lauryloxyacetic acid, decylthioacetic acid or laurylthioacetic acid, and preferably coconut oil fatty acid, e.g. the methyl or ethyl ester of such acid, in the presence of sodium ethanolate or potassium ethanolate, according to the procedure described in British Patent 631,367, with an aliphatic amine, preferably with one of the following:

- (a) Monohydroxy-alkylamines, e.g.,  $\beta$ -hydroxy-ethylamine,  $\gamma$ -hydroxy-propylamine, or di-hydroxy-alkylamines, e.g.  $\beta,\gamma$ -dihydroxy-propylamine;
- (b) Bis-( $\omega$ -hydroxyalkyl)-amines, e.g., bis-( $\beta$ -hydroxyethyl)-amine, bis-( $\gamma$ -hydroxy-propyl)-amine, bis-( $\alpha$ -methyl- $\beta$ -hydroxyethyl)-amine;
- (c) N-alkyl-N-(hydroxyalkyl)-amines, e.g. N-methyl- or N-ethyl-N-( $\beta$ -hydroxyethyl)-amine, or N-methyl- or N-ethyl-N-( $\gamma$ -hydroxypropyl)-amine.

In the definition of amines enumerated above under (a), (b) and (c), "alkyl" represents preferably "lower alkyl" i.e. alkyl of at most 4 carbon atoms.

Most preferred amides are those of amines defined under (b), wherein "alkyl" has from 2 to 3 carbon atoms, and fatty acids, especially the bis-( $\beta$ -hydroxyethyl)-amides and bis-( $\gamma$ -hydroxypropyl)-amides of coconut oil fatty acid, since they assist in obtaining particularly good color yields.

The acid wool dyestuffs usable according to the invention, i.e. the color moiety of which is an anion and which draw from a neutral to acid bath, can be of any class of dyestuffs desired. They can be, for example, metal-free, metallizable or metal-containing azo, anthraquinone, phthalocyanine or nitro dyestuffs, or methine or triphenylmethane dyes. The dyes can be water-soluble basic as well as acid dyes, or water-dispersible dyes. Azo dyes can be mono-, dis- or poly-azo dyes including formazanes, and the complexing metal can be chromium, cobalt, nickel or copper. Metal-containing azo dyestuffs free from sulfonic acid groups are preferred, particularly those which contain two molecules of azo dyestuffs to one metal atom. Suitable metals therein are principally chromium or cobalt.

Polyamide fibers, especially wool, can also be dyed by the process of the invention using chromium dyes, especially chromable azo dyes which latter are used together with salts of trivalent chromium or soluble chromates in acid medium. Furthermore, fiber reactive dyestuffs, especially fiber-reactive-azo, anthraquinone or phthalocyanine dyestuffs can be used.

Polyester fibers are dyed according to the invention preferably with dispersible dyes, while acrylic fibers are preferably dyed with aqueous solutions of suitable basic dyes, e.g. methine, azomethine, diphenylmethane or triphenylmethane dyes or with arylazo or anthraquinone dyes having an external onium group.

Suitable products known in textile printing are used as thickeners, in particular the water soluble salts of alginic acid, galactomannan, tragacanth, British gum or locust bean flour. However, cellulose derivatives such as methyl cellulose or carboxymethyl-cellulose can also be used.

Formation of deposits in the dye liquors must, of course, be avoided.

Material made of both synthetic and natural polyamides can be used as polyamide fibers which can be dyed according to the invention. Examples of natural polyamides are wool and silk; examples of synthetic polyamides are nylon 6 (Perlon), nylon 66 and nylon 16. Polyester fibers such as cellulose diacetate, cellulose triacetate, high-molecular esters of aromatic polycarboxylic acids and polyhydric alcohols, e.g. poly-(ethylene glycol polyterephthalate), as well as acrylic acids and methacrylic homopolymeric and copolymeric fibers can also be dyed by the process according to the invention. In the case of synthetic polyamides drying under thermo-fix conditions after the impregnation is favourable. The dyeing process according to the invention is principally used for wool. The fibrous material can be dyed according to the invention in any form, for example, in the form of loose stock, slubbings, tops, tow, worsted, yarn or fabrics. It can also be in the form of blended fibers, e.g. of polyamide and incrusted cellulose fibers, or in the form of mixed fabrics, e.g. of wool and polyester fibers mentioned above. It is thus possible to dye only one of the fiber compounds, e.g. the polyamide fibers, or both compounds simultaneously, by dyestuffs suitable for such dyeing.

The polyamide material is impregnated by printing, coating or spraying, but preferably by treatment in the pad-mangle. The impregnation liquor as defined is advantageously prepared by first dissolving the dyestuff in an about 80° C. warm aqueous solution containing the fatty acid di- and/or tri-alkanolamine condensation product, the tetrahydronaphthalene sulfonic acid and, optionally, thioglycolic acid, and advantageously also thickeners as well as, if desirable, triethanolamine, diluting this solution with cold water up to the desired concentration, care being taken that the temperature of the liquor does not rise above about 40° C. The impregnation liquor should contain about 5 to 100 g./liter of the mixtures of assistants (1) and (2), and preferably about 10-60 g./liter of color transfer agent (1), e.g. fatty acid polyalkanolamine condensation product, 2-20 g./liter of "blowing" control agent (2), e.g.  $\beta$ -tetrahydronaphthalenesulfonic acid or a mixture of  $\alpha$ - and  $\beta$ -tetrahydronaphthalenesulfonic acid and, if necessary, 0.1 to 3 g./liter of thioglycolic acid, the ratio of color transfer agent to "blowing" control agent, as indicated by the foregoing proportions, being in most cases within the range of 1.5:1 to 5:1, but preferably about 1.5:1 to 4:1, optimal results being obtained at about 2.5:1 to 3:1. The polyamide material is impregnated advantageously under 40° C. and then wrung out. The content of impregnating liquor should be about 40 to 110%, and not more than 130% of the dry weight of the fibers. Impregnation of polyamide material is preferably carried out at about 30° to 70° C.

Application of about 0.5 to 10% of the additive mixture of (1) and (2) calculated on the dry weight of the goods to be dyed, is thus recommended.

Apart from thioglycolic acid or its water-soluble salts, the use of which agents is recommended mainly when dyeing synthetic polyamide fibers, there may also be used other agents having a swelling effect on the fibers, such as o-phenylphenol, especially when dyeing polyterephthalate type fibers.

Solvents such as ethylene glycol monomethyl ether, or monoethyl ether (Cellosolve), thiodiethylene glycol, isopropanol or butanol, and wetting agents such as succinic acid-sulfo succinate may be added to the dye liquor as conventional adjuvants, in amounts of about 3 to 20 g. and preferably of 5 to 10 g., per liter of dye liquor.

Pad liquors according to the invention are prepared conveniently from pre-mixed, concentrated dye compositions which consist essentially of:

- 5 (a) 8 to 35 and preferably 10 to 20% by weight of dyestuff, especially a dyestuff of the kind described further below,
- 10 (b) 5 to 35% by weight of a mixture of color transfer agent and "blowing control" agent as defined hereinbefore, the balance of the dye composition consisting of
- 15 (c) water,
- 20 (d) 0 to 5% by weight, depending on the kind of dyestuff present, of an acidic agent, preferably acetic acid, formic acid, sulfuric acid or phosphoric acid, and, optionally, an aqueous thickener, preferably galactomannan or locust bean flour, and
- 25 (e) isopropanol, or butanol and/or  $\beta$ -alkoxyalkanol, in order to impart to the dye composition a viscosity of about 1 to 50, and preferably 10 to 40 poise, all percentages being calculated on the total weight of the composition.

Dye liquors according to the invention are prepared from such concentrated dye compositions, by adding to 100 to 400 g. of the latter sufficient water and/or aqueous thickener solution to obtain one liter of dye liquor, the degree of dilution depending on the desired color depth of the resulting dyeings.

The impregnated polyamide material is steamed by the usual methods, advantageously with neutral saturated steam. Wool and silk are steamed at about 100-120° C., synthetic fibers at about 100-140° C. Synthetic polyamide and polyester fibers can also be thermofixed by heating in a dry medium to 150 to 250° C.

When padding is done with a dye-liquor having a pH above 4 or 4.5 the dyestuff is subsequently fixed on the polyamide material by treatment in a hot acid bath having a pH in the range of about 2 to 3 by known methods. Advantageously the goods are introduced into the acid bath at 80-98° C. Acids suitable for the acid bath are inorganic and organic acids as well as acid salts. Examples of inorganic acids are sulphuric acid, phosphoric acid or hydrochloric acid. Examples of organic acids are formic acid or acetic acid; suitable acid salts are, e.g., sodium or potassium hydrogen sulphate or ammonium chloride. Organic acids are preferred, in particular formic acid. In some cases it is also useful to add water-soluble salts, preferably water-soluble calcium salts of mineral acids, in particular calcium chloride, to the acid bath.

After the dyestuff has been fixed on the polyamide material, whether by steaming or by treatment in a hot acid bath, or by thermofixation, the material is rinsed in the usual way, advantageously with an aqueous solution of formic acid or acetic acid, depending on the type of polyamide, at 40-98° C.; detergents may be added to the rinsing liquor.

Compared with previously known processes used for the same purpose, the process for the dyeing of polyamide material according to the invention is distinguished by various advantages. For example, it gives better dyestuff yields, better penetration of the polyamide material and the dyeing is more level on this material; in addition, it is possible to dye penetratively and evenly, woollen goods obtained by mixing wool of different origin, whereby the fastness to light is increased in many cases.

Deep shades can be obtained with very short fixation times, which means that the mechanical strength of the fibers remains essentially unimpaired, contrary to what occurs in longer fixation treatment.

Also the fibers treated according to the invention have a softer feel and can be spun better; the impregnation liquors are easily prepared; especially those prepared with compositions containing components (2) as defined under ( $\alpha$ ) and ( $\beta$ ) have unexpected stability, and they do not substantially soil the apparatus; finally, an intermediate drying of the impregnated goods can be avoided which is a saving in time and apparatus.

One particularly outstanding advantage of the dyeings

produced by the process according to the invention is the essential freedom of these dyeings from the well-known sandwich effect, which is very noticeable as a grey shimmer dulling the brilliance of the shade of dyed fabrics and giving the latter a poor aspect.

The sandwich effect is particularly disturbing in black, blue, green and red shades, while it is less readily detected in yellow and orange shades, unless the fabric is viewed at a relatively flat angle.

In the alkylated anion-active agents listed under (2) above, the lower limit of 8 carbon atoms in the alkyl moiety is critical. For instance, dyeings produced with compositions containing alkyl-benzene-sulfonic acid or dialkyl-benzene-sulfonic acids in which each alkyl substituent has below 8, e.g., 5 or even fewer, carbon atoms as anionic component, show a very pronounced sandwich effect.

Pad liquors according to the invention containing in the composition as component (2) substances as defined under ( $\alpha$ ) and ( $\beta$ ) are homogeneous and particularly stable e.g. against electrolytes, and can be preserved for several days without undue coacervation and formation or irreversible dye deposits in the vessels used for storing the dye liquors, in the case of using control agent (2)( $\alpha$ ), even at pH values in the range below 7, and down to 2.

The dyestuff in these liquors is usually very finely distributed and in a uniform state of dispersion, which facts lead to the above mentioned uniformity and good penetration in the resulting dyeings. Dyestuff mixtures can be used without difficulty.

Moreover, dye liquors according to the invention have the desirable advantage of greatly reduced foam formation during padding while pad liquors containing only component (1), but not component (2) are liable to foam excessively in the pad mangle. Especially, as a consequence of reducing foaming, the "blowing" effect on the padded fibers caused by the subsequent steam treatment, which effect increases the volume especially of padded slubbings or tow of wool and the like fibers, and thus contributes to a thorough and even distribution of the dye on all of the fibers, can be controlled to avoid excessive as well as insufficient "blowing." This is particularly important when steaming is carried out on apparatus which comprises a first pre-steaming zone from which the pre-steamed material is moved downwardly through a narrow, vertically disposed duct or channel into a second steaming zone in which it may arrive in folded condition. The pre-steamed material should pass through the vertical duct portion and optionally be laid into folds therein preferably without coming into contact with any mechanical obstructions that could, among other difficulties, cause breaking of the slubbing or the like foldable material. Excessive voluminosity of the pre-steamed material brought about in the pre-steaming zone may, of course, impede the passage of the material through the above-mentioned duct.

Dyed material obtained according to the process of the invention shows a satisfactorily reduced blowing in the presteaming zone so that it passes readily through the vertical duct of such steaming apparatus. This is particularly surprising in the case of using components as defined under (2)( $\alpha$ ), supra, because such components themselves are well known as foaming agents; nevertheless the combination of these substances with the substances defined under (1), being themselves foam-forming and of excessive blowing effect, affords compositions which lead to a most desirable strong, but very brief blowing of the fiber material in the pre-heating zone itself leading to a voluminousness which recedes immediately so that the material can pass unimpeded through the above-mentioned vertical duct into the second steaming zone.

It is noteworthy that each of the two components of the compositions according to the invention when used alone in the pad-dyeing process under the conditions de-

scribed above causes strong sandwich effects in the dyeings produced as polyamide fibers.

Dyeings produced according to the process of the invention using a pad liquor of low pH and as component (2) some of the substance as defined under (2)( $\gamma$ ), show, when dyed in pastel shades, a tendency to yellow when exposed to sunlight. This is not the case when using condensation products of formaldehyde with naphthalene-sulfonic acid and/or tetrahydro-naphthalene-sulfonic acid, or such condensation products also containing methyl-substituted toluene-benzene-sulfonic acid condensed therewith.

The following non-limitative examples serve to illustrate the invention further. Temperatures are given therein in degrees centigrade. Where not otherwise expressly stated, parts and percentages are given by weight. The relationship of parts by weight to parts by volume is as that of grams to milliliters. C.I. means "Color Index."

#### Example 1

40 parts of the chromium-containing monoazo dyestuff: 2-hydroxy - 5 - sulphomethylamide - 1 amino-benzene  $\rightarrow$  1 - carboethoxyamino - 7 - hydroxynaphthalene (dyestuff:chromium=2:1) are dissolved in an 80° warm mixture consisting of 300 parts of a 2.5% aqueous sodium alginate solution, 30 parts of condensation product of coconut fatty acid and 2 equivalents of diethanolamine (according to Example 3 of U.S. Patent No. 2,089,212) and the solution of 15 parts of the sodium salt of  $\beta$ -tetrahydronaphthalene sulphonic acid in 250 parts of water.

The solution obtained is diluted with about 400 parts of cold water. The temperature of this impregnating liquor should be about 40°.

Wool flannel is impregnated with this liquor at 40°, the goods are wrung out to a liquid content of 80% of the dry weight and then steamed at 102° with saturated steam with a slight excess pressure for 4 minutes. The steamed fabric is then treated in a 98° warm aqueous bath which contains 8 cc./litre of 85% formic acid and then rinsed, first with hot and then with cold water.

A very level grey wool dyeing which has penetrated very well is obtained. It has no so-called sandwich effect.

If the steaming time in the above example is increased to 8, 15, 30 or 60 minutes, then dyeings of more and more colour strength but otherwise of the same value are obtained.

If, in the above example, instead of the sodium salt of  $\beta$ -tetrahydronaphthalene monosulphonic acid, a corresponding amount of the sodium salt of a mixture consisting of  $\alpha$ - and  $\beta$ -tetrahydronaphthalene monosulphonic acid, or of naphthalene monosulphonic acid or of o-xylene monosulphonic acid is used and otherwise the same procedure is followed, then grey dyeings of similar quality are obtained.

If, in the above example, instead of the dyestuff mentioned, other heavy metal-containing monoazo dyestuffs are used, e.g. those of the commercial names Irgalan Olive BGL, Irgalan Brown 7RL, Irgalan Brown 2 GL or Irgalan Yellow 2 RL of J. R. Geigy A.G. Basle, Switzerland and the procedure described above is followed, then wool flannel dyed olive, brown or yellow is obtained. The dyeings have the same good penetration and evenness as that described above.

If instead of 30 parts of the condensation product of coconut fatty acids and 2 equivalents of diethanolamine, 30 parts of the condensation product of coconut fatty acid and 2 equivalents of triethanolamine are used and otherwise the procedure given in the example is followed, then equally good and well penetrated dyeings are obtained.

#### Example 2

Wool flannel is impregnated at 40° with an impregnation liquor produced according to Example 1, first paragraph, and then wrung out to a liquor content of 80% calculated on the dry weight. The fabric which has

been treated in the padding machine is passed through a 98° warm aqueous bath which contains 8 cc. per litre of 85% formic acid at such a rate that the material remains in the bath 5 minutes. There is only inconsiderable bleeding of the dyestuff into the acid bath. The wool flannel so dyed is then washed for 5 minutes with a 45° warm aqueous solution of 0.5 g./litre nonylphenol polyglycol ether, and then rinsed with cold water. The grey dyeing obtained is well dyed through and has no so-called sandwich effect.

Example 3

Wool flannel is treated in the padding machine at 40° with an impregnation liquor which contains the dyestuff Polar Brilliant Blue GAW (C.I. 61135 Acid Blue 127) instead of the metal-containing azo dyestuff mentioned in the first paragraph of Example 1, which liquor is otherwise prepared as described in Example 1, paragraph 1. The material is wrung out to a liquid content of 80% of the dry weight and then steamed for 4 minutes at 102° under slight excess pressure. The goods are then rinsed first with hot and then with cold water.

A very level and well penetrated blue wool dyeing is obtained which has no so-called sandwich effect.

If instead of Polar Brilliant Blue GAW, the dyestuff of the formula

10

A very level and well penetrated yellow silk dyeing is obtained which has no so-called sandwich effect.

On increasing the steaming time in the above example to 8, 15, 30 or 60 minutes yellow silk dyeings of greater and greater colour strength but otherwise having the same properties are obtained.

If in the above example, instead of the dyestuff mentioned, the dyestuff Neolan Yellow 8 GE (C.I. Acid Yellow 101) is used, then yellow silk serge dyeings are obtained of equal penetration and evenness.

If instead of 30 parts of the condensation product of coconut fatty acid and 2 equivalents of diethanolamine, 30 parts of the condensation product of coconut fatty acid and 3 equivalents of diethanolamine are used and otherwise the procedure given in the example is followed, then equally good and well penetrated dyeings are obtained.

Example 6

Silk serge is impregnated at 40° with an impregnation liquor produced according to Example 5, paragraph 1, the goods are wrung out to a liquor content of 80%, and passed through a 98° warm aqueous bath which contains 8 cc./litre of 85% formic acid at such a rate that the material of the dyestuff into the acid bath occurs. The dyed silk serge is then washed with a 45° warm



is used and otherwise the same procedure as described in the example is followed, then equally good and level well penetrated material dyed red is obtained.

Example 4

Wool flannel is impregnated at 40° with an impregnating liquor produced according to Example 3 paragraph 1 and then wrung out to a liquor content of 80% of the weight of the fibres. The padded fabric is then passed through a 98° warm aqueous bath containing 8 cc./litre of 85% formic acid and 2 grams per litre of calcium chloride at such a rate that the material is in the bath for 5 minutes, during which process only inconsiderable bleeding of the dyestuff into the acid bath occurs. The goods are then washed with a 45° warm aqueous solution of 0.5 g./litre phenol polyglycol ether and then rinsed with cold water.

The wool flannel so obtained is well penetrated and the dyeing is very level without any so-called sandwich effect.

Example 5

40 parts of the cobalt-containing monoazo dyestuff: 2-hydroxy-1-aminobenzene-5-sulphonic acid methylamide → 1-phenyl-3-methylpyrazolone (dyestuff:cobalt=2:1) are dissolved in an 80° warm mixture consisting of 300 parts of a 2.5% aqueous sodium alginate solution, 30 parts of the condensation product of coconut fatty acid and 2 equivalent of diethanolamine (according to Example 3 of U.S. Patent No. 2,089,212) and the solution of 15 parts of the sodium salt of  $\beta$ -tetrahydronaphthalene sulphonic acid in 250 parts of water. This solution is diluted with about 400 parts of cold water. The temperature of this impregnation liquor should be about 40°.

Silk serge is impregnated at 40° with this liquor, the goods are wrung out to a liquid content of 80% of the dry weight and steamed with saturated steam for 4 minutes at 102° under slight excess pressure. The fabric is then rinsed first with hot and then with cold water.

40 aqueous solution of 0.5 g./litre nonylphenol polyglycol ether and afterwards rinsed with cold water.

In this way, well penetrated yellow silk serge of good evenness is obtained and there is no so-called sandwich effect.

Corresponding dyeings on silk serge of equally good penetration of the material and evenness of the dyeings are obtained if, instead of the dyestuff mentioned in the above example, Neolan Yellow 8 GE (C.I. Acid Yellow 101) is used and otherwise the procedure given above is followed.

Example 7

37.5 parts of the chromium-containing monoazo dyestuff 2-carboxyl-1-aminobenzene → 1-phenyl-3-methylpyrazolone (dyestuff:chromium=2:1) and 14.0 parts of the chromium-containing monoazo dyestuff 2-hydroxy-5-sulphomethylamido-1-aminobenzene → 1-carboethoxyamino-7-hydroxynaphthalene (dyestuff:chromium=2:1) are dissolved in an 80° warm mixture of 300 parts of a 2.5% aqueous sodium alginate solution, 10 parts of the condensation product of coconut fatty acid and 2 equivalents of diethanolamine, 20 parts of triethanolamine, a solution of 15 parts of the sodium salt of  $\beta$ -tetrahydronaphthalene sulphonic acid and 270 parts of water and the solution obtained is diluted with about 400 parts of cold water. The temperature of this impregnation liquor should be about 40°.

Nylon canvas is impregnated with this liquor, wrung out to a liquid content of 50%, steamed for 8 minutes at a temperature of 130° and then rinsed first with hot and then with cold water.

70 A very well penetrated and very level olive dyeing is obtained which has no so-called sandwich effect.

Example 8

75 Nylon canvas is impregnated at 40° with an impregnation liquor produced according to Example 8, paragraph 1.

11

The goods are then wrung out to a liquid content of 50% and passed through a 98° warm aqueous bath which contains 4 cc. per liter of 85% formic acid at such a rate that the material remains in this bath for 4 minutes. Only an inconsiderable bleeding of the dyestuff into the acid bath occurs. The nylon canvas so dyed is then rinsed first with warm and then with cold water.

The nylon canvas so obtained is well penetrated and evenly dyed olive green.

### Example 9

Canvas made of poly- $\epsilon$ -aminocapro lactam (Perlon) is impregnated at 40° with an impregnation liquor produced according to Example 7. The goods are then wrung out to a liquor content of 50% and dried under thermo-fix conditions for 45 seconds at 190°.

The Perlon canvas so impregnated is then passed through a 98° warm aqueous bath which contains 4 cc./litre of 85% formic acid and is treated for 4 minutes at the boil in this bath. It is then rinsed with warm and then cold water.

The Perlon canvas so treated is well penetrated and a level olive dyeing is obtained.

### Example 10

The orange-red worsted yarn so dyed is well penetrated and the dyeing is very level. The feel of the goods is very pleasant and voluminous and they can be well combed and spun. Also after the impregnation of liquor has been left standing for weeks, level and penetrated worsted yarn 55 is obtained.

### Example 11

40 parts of chromium-containing monoazo dyestuff: 2 - hydroxy-5-sulphomethylamido - 1 - aminobenzene → 1 - carboethoxy - amino - 7 - hydroxynaphthalene (dyestuff: chromium = 2:1) are stirred in a solution produced according to Example 1, paragraph 1, but containing 500 parts of sodium alginate solution instead of 300 parts.

1. Woolen worsted yarn is printed in the manner usual for vigoureux printing with this liquor with a liquor take-up of 85%. The printed goods are after-treated by steaming and rinsing as described in Example 10. Grey coloured woolen worsted yarn is obtained which is distinguished by a full, voluminous feel. The goods can be well combed and spun.

### Example 12

80 parts of Eriochrome Black A (C.I. 15710) are dissolved in a 60° warm mixture of 300 parts of a 2.5% sodium alginate solution and 30 parts of a mixture of

12

the condensation product of coconut fatty acid and 2 equivalents of diethanolamine (according to U.S. Patent No. 2,089,212, Example 3) and the solution of 30 parts of the sodium salt of  $\beta$ -tetrahydronaphthalene sulphonic acid in 250 parts of water, and also 10 parts of potassium chloride in 100 parts of water. The solution is then made up to 1000 parts with water; the temperature should be 40°.

be 40°. Woolen slubbing is impregnated with this liquor at 10 40°, wrung out to a liquor content of about 80% and steamed with saturated steam at 98° for 1 hour. It is then rinsed with an aqueous solution of 0.5 g./litre of a condensation product according to U.S.P. 2,089,212 in a back washing machine, rinsed with about 30° warm water and 15 then acidified in a new bath with an aqueous 30° warm solution of 0.2 cc./litre or 85% formic acid. Finally the goods are again rinsed with 30° warm water.

Woollen slubbing dyed a level black is obtained which can be well combed and spun.

Similar level-dyed woollen slubbings of vivid brownish-red shade are obtained by repeating Example 12, but using in lieu of the dyestuff employed therein, 50 parts of a dyestuff being a mixture of the orange 2:1 chromium complex of the dyestuff of the formula



### the red dyestuff of the formula



and the blue dyestuff of the formula



in a weight ratio of 25:25:6.

### Example 13

65 40 parts of the chromium-containing monoazo dye  
stuff: 2-hydroxy-5-sulphomethylamido-1-aminobenzene->  
carboethoxyamino-7-hydroxynaphthalene (dyestuff:chromium=2:1) are dissolved in an 80° warm mixture con-  
sisting of 300 parts of a 2.5% aqueous sodium alginate  
70 solution and 30 parts of condensation product of coconut  
fatty acid and 2 equivalents of diethanolamine (accord-  
ing to Example 3 of U.S. Patent 2,089,212) and the  
solution of 15 parts of sodium salt of  $\beta$ -tetrahydronaph-  
thalene sulphinic acid and 2 parts of thioglycolic acid in  
75 250 parts of water. The solution obtained is diluted with

400 parts of cold water. The temperature of the solution should be about 40°.

Wool flannel is impregnated with this liquor at 40°, the



dyeing is obtained which has no so-called sandwich effect.

If instead of Polar Brilliant Blue GAW, the dyestuff of the formula



goods are wrung out to a liquid content of 80% of the dry weight and then steamed at 102° with saturated steam with a slight excess pressure for 4 minutes. The fabric is then rinsed first with hot and then with cold water.

A very level grey wool dyeing which has penetrated very well is obtained. It has no so-called sandwich effect.

If the steaming time in the above example is increased to 8, 15, 30 or 60 minutes, then dyeings of more and more colour strength but otherwise of the same value are obtained.

If in the above example, instead of the 15 parts of the sodium salt of  $\beta$ -tetrahydronaphthalene sulphonic acid, the same number of parts of a mixture of sodium salt of  $\alpha$ - and  $\beta$ -tetrahydronaphthalene sulphonic acid or of solution salt of o-xylene sulphonic acid or 30 parts of sodium salt of naphthalene sulphonic acid are used and otherwise the same procedure as described in the example is followed, then dyeings having similar qualities are obtained.

If in the above example instead of the dyestuff mentioned, other heavy metal-containing monoazo dyestuffs are used, e.g. those of the commercial names Irgalan Olive, BGL, Irgalan Brown 7 RL, Irgalan Brown 2 GL or Irgalan Yellow 2 RL and the procedure described above is followed, then wool flannel dyed olive, brown or yellow is obtained. The dyeings have the same good penetration and evenness as that described above.

If instead of 30 parts of the condensation product of coconut fatty acid and 2 equivalents of diethanolamine, 30 parts of the condensation product of coconut fatty acid and 1 equivalent of triethanolamine are used and otherwise the procedure given in the example is followed, then equally good and well penetrated dyeings are obtained.

#### Example 14

Wool flannel is impregnated at 40° with an impregnation liquor produced according to example 13, first paragraph and then wrung out to a liquor content of 50% calculated on the dry weight. The fabric which has been treated in the padding machine is passed through a 98° warm aqueous bath which contains 8 cc. per litre of 85% formic acid at such a rate that the material remains in the bath 5 minutes. There is only an inconsiderable bleeding of the dyestuff into the acid bath. The wool flannel so dyed is then washed for 5 minutes with a 45° warm aqueous solution of 0.5 g./litre nonylphenol polyglycol ether, and then rinsed with cold water. The grey dyeing obtained is well dyed through and has no so-called sandwich effect.

#### Example 15

Wool flannel is treated in the padding machine at 40° with an impregnation liquor which contains the dyestuff Polar Brilliant Blue GAW (C.I. 61135 Acid Blue 127) instead of the metal-containing azo dyestuff mentioned in the first paragraph of Example 13, which liquor is otherwise prepared as described in Example 13, paragraph 1. The material is wrung out to a liquor content of 80% of the dry weight and then steamed for 4 minutes at 102° under slight excess pressure. The goods are then rinsed first with hot and then with cold water.

A very level and well penetrated blue wool flannel 75

15 or Neolan Yellow 8 GE (C.I. Acid Yellow 101) is used and otherwise the same procedure as described in the example is followed, then equally good and level well penetrated material dyed red or yellow respectively is obtained.

#### Example 16

20 Wool flannel is impregnated at 40° with an impregnating liquor produced according to Example 15 paragraph 1 and then wrung out to a liquor content of 80% of the weight of the fibres. The padded fabric is then passed through a 98° warm aqueous bath containing 8 cc./litre of 85% formic acid at such a rate that the material is in the bath for 5 minutes, during which process only inconsiderable bleeding of the dyestuff into the acid bath occurs. The goods are then washed with a 45° warm aqueous solution of 0.5 g./litre nonylphenol polyglycol ether and then rinsed with cold water.

25 The wool flannel so obtained is well penetrated and the blue dyeings are very level without any so-called sandwich effect.

#### Example 17

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545

able bleeding of the dyestuff into the acid bath occurs. The dyed silk serge is then washed with a 45° warm aqueous solution of 0.5 g./litre nonylphenol polyglycol ether and afterwards rinsed with cold water.

In this way, well penetrated yellow silk serge of good evenness is obtained and there is no so-called sandwich effect.

Corresponding yellow dyeings on silk serge of equally good penetration of the material and evenness of the dyeings are obtained if, instead of the dyestuff mentioned in the above example, Neolan Yellow 8 GE (C.I. Acid Yellow 101) is used and otherwise the procedure given above is followed.

#### Example 19

In order to prepare a pad liquor

(a) 40 parts of Eriochrome Black A (C.I. 15710), 24 parts of which are diluting agent (coupage), are pasted with 40 parts of water of 25°, then there are added to the paste with stirring 750 parts of water having a temperature of 60°, 7 parts of galactomannan thickener pasted with 10 parts of ethanol; the resulting liquor is heated to the boil for 2 to 3 minutes and then left to cool to about 40°;

(b) 20 parts of 85% formic acid, 25 parts of chromium trifluoride and 60 parts of water of 20° are mixed and the resulting slurry is added to the foregoing liquor;

(c) 30 parts of a condensation product of coconut oil fatty acid and 2 equivalents of diethanolamine prepared according to Example 3 of U.S. Patent 2,089,212, and 20 parts of sodium 4-(1-methyl-undecyl)-benzene-1-sulfonate (or the product containing the latter which is commercially available under the tradename of Marlon A 375) are mixed with 50 parts of water, and

(d) 50 parts of the mixture resulting from (c) are added to the acidified liquor obtained by step (b), supra. Water is then added to the resulting composition to adjust the total volume of the dye liquor to 1000 parts. This pad liquor is very stable and can be left standing for several days without undue conservation.

(e) Woollen slubbing is impregnated with this liquor at 40°, wrung out to a liquor content of about 80% and steamed with saturated steam at 98° for 1 hour. It is then rinsed with an aqueous solution of 0.5 g./liter of sodium dodecyl-benzenesulfonate in a back washing machine at 40°, and then rinsed with about 30° warm water and left to dry.

Woollen slubbing dyed a level black free from sandwich effect is obtained which can be well combed and spun.

When steamed on a two-phase steaming machine having a first pre-steaming zone above a narrow vertical duct for the pre-steamed material and a subsequent large horizontal steaming zone into which the lower exit of the duct opens, the slubbing is "blown" strongly but only very briefly while in the presteaming zone above the vertical zone, but the luminousness due to the "blowing" effect recedes promptly so that the slubbing passes through the vertical duct unimpeded.

By using in step (c) of the above Example 19, instead of sodium dodecyl-benzenesulfonate an equivalent amount of potassium p-(1,3,3,5 - tetramethyl-octyl)-benzene-sulfonate, di(β-hydroxyethyl)-ammonium p-(1 - methyl-octyl)-benzene-sulfonate, or 1,2 - di-[4 - sulfo-naphthyl-(2)]-ethane, or a condensation product of a mixture of xylene sulfuric acid and naphthalene sulfuric acid (molar ratio 5:4) with 1.7 equivalents of formaldehyde, and otherwise following the same procedure as described in Example 19, then black dyeings of similar quality are obtained.

If instead of 30 parts of the condensation product of coconut oil fatty acid and 2 equivalents of diethanolamine, 40 or 60 parts of the condensation product of coconut oil fatty acid and 2 equivalents of triethanolamine or of 30, 40, or 60 parts of coconut oil fatty acid diethanolamide, respectively, are used in step (c), supra, and otherwise the

procedure given in Example 19 is followed, then equally satisfactory dyeings are obtained.

Similar satisfactory black dyeings are obtained when repeating Example 19, but using in step (c) in lieu of the 30 parts of the condensation product used therein, 25 parts of the same condensation product, an in lieu of 20 parts of the sodium salt of methylundecylbenzene sulfonic acid used therein, 10 parts of the sodium salt of the condensation product obtained from 2 equivalents of naphthalene-sulfonic acid and 1.4 equivalents of formaldehyde or 10 parts of the sodium salt of the condensation product of:

- (a) 2 equivalents of naphthalene-sulfonic acid and 1.5 parts of acetaldehyde; or
- (b) 1 equivalent of naphthalene-sulfonic acid, 1 equivalent of tetrahydronaphthalene-sulfonic acid, and 1.5 equivalents of paraformaldehyde; or
- (c) 1 equivalent of naphthalene-sulfonic acid, 1 equivalent of methylnaphthalene-sulfonic acid, and 1.9 equivalents of formaldehyde.

Similar level-dyed woollen slubbings of vivid brownish-red shade are obtained by repeating Example 19, but using in lieu of the dyestuff employed therein, 50 parts of a dyestuff being a mixture of:

- (i) the orange 2:1 chromium complex of the dyestuff of the formula



- (ii) the red dyestuff of the formula



- (iii) and the blue dyestuff of the formula



in a weight ratio of 25:25:6, omitting the chromium trifluoride, and using 15 in lieu of 20 parts of aqueous 85% formic acid in the preparation of the pad liquor.

#### Example 20

Wool flannel is impregnated at 40° with an impregnation liquor produced according to step (c) of Example 19, and then wrung out to a liquor content of 100% calculated on the wool dry weight. The fabric which has been treated in the foulard is passed through a 98° warm aqueous bath which contains 8 ml per liter of 85% formic acid at such a rate that the material remains in the bath for

30 minutes. There is only a negligible amount of bleeding of the dyestuff into the acid bath. The wool flannel so dyed is then washed for 5 minutes with a 45°-warm aqueous solution of 0.5 g/liter nonylphenol polyglycol ether, and then rinsed with cold water. The grey dyeing obtained is well-penetrated and has no so-called sandwich effect.

## Example 21

A pad liquor is prepared as described in Example 19, but using in lieu of the 40 parts of black dye employed therein, only 5 parts of the chromium-container mono-azo dyestuff obtained by coupling diazotized 2-hydroxy-5-N-methyl-sulfamyl-1-amino-benzene with 1-ethoxycarbonylamino-7-hydroxynaphthalene and chroming the resulting metallizable azo dye with chromium chloride in a molar ratio of dyestuff to metal of 2:1, and adding 25 parts of aqueous 80% acetic acid in lieu of the formic acid employed in Example 19.

20 parts of the auxiliary mixture prepared as described in Example 19(c) are added in lieu of the 25 parts used in Example 19(d).

The pad liquor thus obtained is stable for several days.

Wool flannel is impregnated with this resulting liquor at 40°, the goods are wrung out to a liquid content of 100% of the dry weight and then steamed at 102° with saturated steam with slight excess pressure for 20 minutes. The steamed fabric is then rinsed, first with hot and then with cold water.

A very level wool dyeing of grey pastel shade which has penetrated very well is obtained. It has no sandwich effect.

If the steaming time in the above example is increased to 30 or 60 minutes, then dyeings of greater color strength but otherwise of the same quality are obtained.

## Example 22

Similar results are obtained by repeating Examples 19, 20 and 21, respectively, but using in each case in lieu of the auxiliary mixture produced as described in step (c) of Examples 19, 30, 40 or 60 parts, respectively, of an auxiliary mixture prepared from the following components:

(a)

40 parts of coconut oil fatty acid N,N-di-( $\beta$ -hydroxyethyl)-amide,  
10 parts of diethanolammonium p-dodecyl-benzene-sulfonate,  
50 parts of water;

(b)

35 parts of the same condensation product as used in Example 19 (c),  
15 parts of sodium p-(1,3,3,5-tetramethyl-octyl)-benzene sulfonate,  
2 parts of isopropanol;

(c)

20 parts of the same condensation product as used in Example 19 (c),  
20 parts of coconut oil fatty acid N,N-di-( $\beta$ -hydroxyethyl)-amide,  
15 parts of diethanolammonium p-(1-methyl-octyl)-benzene-sulfonate,  
55 parts of water;

(d)

25 parts of the same condensation product as used in Example 19 (c),  
25 parts of diethanolammonium p-nonylphenol-sulphonate,  
45 parts of water;

(e)

25 parts of coconut oil fatty acid diethanolamide,  
5 parts of potassium p-(1,3,3,5-tetramethyl-octyl)-benzenesulfonate,  
30 parts of water;

(f)

20 parts of coconut oil fatty acid N,N-di-( $\beta$ -hydroxyethyl)-amide,  
20 parts of sodium dodecyl-naphthalene-sulfonate,  
35 parts of water;

(g)

20 parts of lauric acid N-( $\beta$ -hydroxy-propyl)-amide,  
10 parts of ammonium decylnaphthol-sulfonate,  
35 parts of water;

(h)

20 parts of capric acid N,N-( $\gamma$ -hydroxy-propyl)-amide,  
15 parts of ammonium p-decylbenzene-sulfonate,  
35 parts of water;

(i)

20 parts of coconut oil fatty acid N,N-di-( $\beta$ -hydroxyethyl)-amide,  
20 parts of sodium dodecyl-naphthalene-sulfonate,  
4 parts of n-butanol,  
35 parts of water;

(j)

25 parts of the same condensation product as used in Example 19 (c),

25 parts of diethylammonium p-nonylphenol-sulphonate,  
3 parts of n-butanol;

(k)

30 parts of coconut oil fatty acid N-methyl-N- $\beta$ -hydroxyethyl-amide,

10 parts of sodium salt of the condensation product of 1 equivalent of naphthalene-sulfonic acid, 1 equivalent of methylnaphthalene sulfonic acid and 1.6 equivalents of formaldehyde,

2 parts of isopropanol;

(l)

40 parts of coconut oil fatty acid N,N-di-( $\beta$ -hydroxyethyl)-amide,

10 parts of diethanolammonium salt of the condensation product from: 1 equivalent of benzene-sulfonic acid, 1 equivalent of naphthalene-sulfonic acid and 1.4 equivalents of formaldehyde;

(m)

35 parts of coconut oil fatty acid N,N-di-( $\beta$ -hydroxyethyl)-amide,

15 parts of sodium salt of the condensation product from: 1 equivalent benzene-sulfonic acid, 1 equivalent of naphthalene-sulfonic acid and 1.4 equivalents of glyoxal;

(n)

20 parts of coconut oil fatty acid N,N-di-( $\beta$ -hydroxyethyl)-amide,

20 parts of diethanolammonium salt of the condensation product from: 1 equivalent of toluene-sulfonic acid, 1 equivalent of naphthalene-sulfonic acid and 1.4 equivalents of formaldehyde;

(o)

25 parts of coconut oil fatty acid N,N-di-( $\beta$ -hydroxyethyl)-amide,

25 parts of the sodium salt of the condensation product from: 1 equivalent of benzene-sulfonic acid, 1 equivalent of tetrahydronaphthalene-sulfonic acid and 1.6 equivalents of formaldehyde;

(p)

25 parts of coconut oil acid N,N-di-( $\beta$ -hydroxyethyl)-amide,

5 parts of potassium salt of the condensation product from: 2 equivalents of tetrahydronaphthalene-sulfonic acid and 1.5 equivalents of formaldehyde;

19

(q)

20 parts of coconut oil fatty acid N,N-di-( $\beta$ -hydroxyethyl)-amide,

20 parts of the sodium salt of the condensation product from: 1 equivalent of xylene-sulfonic acid, 1 equivalent of tetrahydronaphthalene-sulfonic acid and 1.7 equivalents of formaldehyde;

(r)

20 parts of lauric acid N,N-di-( $\beta$ -hydroxy-propyl)-amide, 10 parts of the ammonium salt of the condensation product from: 1 equivalent of toluene-sulfonic acid, 1 equivalent of tetrahydronaphthalene-sulfonic acid and 1.6 equivalents of formaldehyde;

(5)

20 parts of capric acid N,N-di-( $\gamma$ -hydroxy-propyl)-amide, 15 parts of the ammonium salt of the condensation product from: 1 equivalent of xylene-sulfonic acid, 1 equivalent of naphthalene-sulfonic acid and 1.5 equivalents of formaldehyde:

(t)

20 parts of coconut oil fatty acid N,N-di-( $\beta$ -hydroxyethyl)-amide.

20 parts of the sodium salt of the condensation product from: 2 equivalents of naphthalene-sulfonic acid and 1.7 equivalents of glyoxal.

### Example 23

Wool flannel is treated in the foulard at 40° with an impregnation liquor which contains 20 parts of the dye-stuff Polar Brilliant Blue GAW (C.I. 61135, Acid Blue 127) instead of Erichrome Black A and is otherwise prepared as described in Example 19 (a) to (d). The material is wrung out to a liquid content of 80% of the dry weight and then steamed for 15 minutes at 102° under slight excess pressure. The goods are then rinsed first with hot and then with cold water.

A very level and well penetrated blue wool dyeing is obtained which is free from sandwich effect.

If instead of Polar Brilliant Blue GAW, the dyestuff of the formula



is used and otherwise the same procedure as described in the example is followed, then equally level and well penetrated material of red shade is obtained.

### Example 24

Example 24  
 40 parts of the chromium-containing monoazo dyestuff: 2-hydroxy-5-methylsulfonyl-1-aminobenzene  $\rightarrow$  1-phenyl-3-methyl-5-pyrazolone (dyestuff:chromium = 2:1) are dissolved in a 60° warm mixture containing of 300 parts a 2.5% aqueous locust bean flour solution and a solution of 30 parts of a mixture consisting of coconut oil fatty acid diethanol-amide and sodium 4-(1-methyl-undecyl)-benzene-sulfonate (weight ratio 1:1) in 250 parts of water. The solution obtained is diluted with 50° warm water to 900 parts by volume and the pH of the solution is adjusted to 2.5. The temperature of the solution should be about 50°. Finally, water is added to make the volume of the liquor up to one liter.

Wool flannel is impregnated with this liquor at 50°, the goods are wrung out to a liquid content of about 100% of the dry weight and then steamed at 98° with saturated steam for 15 minutes. The wool flannel so dyed is then first washed for 5 minutes with a 45° warm aqueous solution of 0.5 g./liter nonylphenol polyglycol either, and then with an aqueous solution containing 2 parts by volume of 85%-formic acid per liter, whereupon it is

20

rinsed with cold water. The orange dyeing obtained is well penetrated and level and has no sandwich effect.

A similar satisfactory result is obtained when repeating the above example but using in lieu of the sodium methylundecylbenzene-sulfonate an equal amount of the sodium salt of the condensation product from 2 equivalents of naphthalene-sulfonic acid and 1.4 equivalents of formaldehyde.

By repeating Example 24, but using 40 parts of a 2:1 dyestuff chromium complex of one of the dyestuffs listed below, in lieu of the dyestuff used therein, then dyeings on wool flannel of similar good quality and the shades given in the right-hand column below are obtained.

|    |                                                                                      | Shade of<br>wool flannel |
|----|--------------------------------------------------------------------------------------|--------------------------|
| 15 | (a)                                                                                  | Red.                     |
| 20 |    |                          |
| 25 | (b)                                                                                  | Navy blue.               |
| 30 |    |                          |
| 35 | (c)                                                                                  | Yellow.                  |
| 40 | (d)                                                                                  | Grey.                    |
| 45 |   |                          |
|    |  |                          |

Similar level-dyed wool flannel of vivid shades are obtained by repeating Example 24, but using in lieu of the 30 parts of dyeing assistant employed therein, 30 parts of a mixture prepared from:

- (i) 50 parts of coconut oil fatty acid diethanolamide and
  - (ii) 50 parts of ammonium p-nonylphenol-sulfonate, or  
in lieu of the latter component, (ii), equivalent amounts  
of di-ethanol-ammonium or triethanol-ammonium 4-(1-  
methyl-undecyl)-benzenesulfonate, or of the ammonium  
salt of the condensation product from 2 equivalents of  
xylene-sulfonic acid (commercial product) and 1.2  
equivalents of formaldehyde.

65 or of the diethanol-ammonium salt or the triethanol-ammonium salt of the condensation product from 2 equivalents of naphthalene-sulfonic acid and 1.4 equivalents of formaldehyde.

### Example 25

- 70 4 parts of the cobalt-containing monoazo dyestuff: 2-hydroxy-1-aminobenzene-5-sulphonic acid methylamide → 1-phenyl-3-methylpyrazolone (dyestuff:cobalt = 2:1) are dissolved in an 80°-warm mixture consisting of 300 parts of water, 7 parts of galactomannan thickener, 15 parts of coconut oil fatty acid diethanolamide and the

## 21

solution of 10 parts of sodium 4-(1-methyl-undecyl)-benzene-1-sulfonate in 250 parts of water. The resulting solution is diluted with about 400 parts of cold water, and 20 parts of 85%-formic acid are added thereto. The temperature of the solution should be about 40°.

Silk serge is impregnated at 40° with this liquor, the goods are wrung out to a liquid content of 80% of their dry weight and steamed with saturated steam for 4 minutes at 102° under slight excess pressure. The fabric is then rinsed first with hot and then with cold water.

A very level and well penetrated yellow silk dyeing is obtained which is free from sandwich effect.

On increasing the steaming time in the above example to 30 or 60 minutes, yellow silk dyeings are obtained which are of greater color strength but otherwise have the same good properties.

If in the above example, instead of the dyestuff mentioned, the dyestuff of the formula



is used, then yellow silk serge dyeings are obtained which are of equal good penetration and evenness.

If instead of coconut oil fatty acid diethanolamide, 30 parts of the condensation product of coconut fatty acid and 3 equivalents of diethanolamine are used and otherwise the procedure given in the example is followed, then equally good and well penetrated dyeings are obtained.

## Example 26

Silk serge is impregnated at 40° with an impregnation liquor produced according to Example 5 but using composition (d) of Example 24 as auxiliary, the goods are wrung out to a liquid content of 80%, and passed through a 98° warm aqueous bath which contains 8 ml./liter of 85% formic acid at such a rate that the material is in the bath for 5 minutes, during which process only inconsiderable bleeding of the dyestuff into the acid bath occurs. The dyed silk serge is then washed with a 45° warm aqueous solution of 0.5 g./liter of nonylphenol polyglycol ether and afterwards rinsed with cold water.

In this way, well penetrated orange-yellow silk serge of good evenness is obtained and there is no so-called sandwich effect.

Corresponding dyeings on silk serge of equally good penetration of the material and evenness of the dyeings are obtained if, instead of the dyestuff mentioned in the above example, Neolan Yellow 8 GE (C.I. Acid Yellow 101) is used and otherwise the procedure given above is followed.

## Example 27

37.5 parts of the chromium-containing monoazo dyestuff - 2 - carboxy - 1 - aminobenzene → 1-phenyl-3-methylpyrazolone (dyestuff:chromium=2:1) and 14.0 parts of the chromium-containing monoazo dyestuff 2 - hydroxy-5 - sulphonethylamido - 1 - aminobenzene → 1-carboethoxyamino - 7 - hydroxynaphthalene

(dyestuff:chromium=2:1)

are incorporated in lieu of Eriochrome Black A into a pad liquor which is otherwise prepared as described in Example 19, but with Composition (c) of Example 22 as auxiliary.

Nylon fabric is impregnated with this liquor wrung out to a liquid content of 50%, steamed for 8 minutes at a temperature of 130° and then rinsed first with hot and then with cold water.

A very well penetrated and very level olive dyeing is

## 22

obtained which is free from sandwich effect and has all the other advantageous properties described hereinbefore.

## Example 28

5 Nylon canvas is impregnated at 40° with an impregnation liquor produced according to Example 22, but with the dyestuff employed in Example 8 and using composition (a) of Example 22 as auxiliary. The goods are then wrung out to a liquid content of 50% and passed through a 98° warm aqueous bath which contains 4 ml. per liter of 85% formic acid at such a rate that the material remains in this bath for 4 minutes. Only an inconsiderable bleeding of the dyestuff into the acid bath occurs. The nylon canvas so dyed is then rinsed first with warm and then with cold water.

10 The nylon canvas so obtained is well penetrated and evenly dyed olive green.

15 When using in lieu of the dyestuff of Example 8, 40 parts of the dyestuff of Example 24, but following otherwise the procedure given above, nylon canvas of similar good quality and orange shade is obtained.

## Example 29

20 Canvas made of poly - ε - aminocaprolactam (Perlon) is impregnated at 40° with an impregnation liquor produced according to Example 23 but using the composition (a) of Example 22 as dyeing auxiliary. The goods are then wrung out to a liquid content of 50% and dried under thermo-fixing conditions for 45 seconds at 190°.

25 The Perlon canvas so impregnated is then passed through a 98° warm aqueous bath which contains 4 ml./liter of 85% formic acid and is treated for 4 minutes at the boil in this bath. It is then rinsed with warm and then cold water.

30 The Perlon canvas so treated is well penetrated and a level yellow dyeing is obtained.

## Example 30

35 2.5 parts of the chromium-containing monoazo dyestuff 2 - carboxy - 1 - aminobenzene → 1-phenyl-3-methylpyrazolone (dyestuff:chromium=2:1) and 0.5 part of the chromium-containing monoazo dyestuff: 2 - hydroxy-5-nitro-1-aminobenzene → 1 - phenyl - 3 - methyl-pyrazolone (dyestuff:chromium 2:1) are incorporated in lieu of Eriochrome Black A into a pad liquor which is otherwise as described in Example 19.

40 Wool slubbing is impregnated at 40° with this liquor, wrung out of a liquid content of 103% of the dry weight and then steamed for 8½ minutes at 104° with saturated steam under slight excess pressure. The goods are then washed with a solution containing 1 g./liter of nonylphenol polyglycol ether and 1 ml./liter of concentrated ammonia solution, then rinsed with water, then washed with an aqueous solution containing 2 ml./liter of 85% formic acid and, if desired, again rinsed with water.

45 The orange-red slubbing so dyed is well penetrated and the dyeing is very level. The feel of the goods is very pleasant and voluminous and they can be well combed and spun. Even after the impregnation liquor has been left standing for several weeks, level and well-penetrated slubbings are obtained therewith.

## Example 31

50 40 parts of chromium-containing monoazo dyestuff: 2 - hydroxy - 5 - sulphonethylamido - 1 - aminobenzene → 1 - carboethoxyamino - 7 - hydroxynaphthalene (dyestuff:chromium=2:1) are stirred in a solution produced according to Example 1, paragraph 1, but containing 500 parts of sodium alginate solution instead of 300 parts.

55 Woollen slubbing is printed in the manner usual for vigoureux printing with this liquor with a liquor take-up of 85%. The printed goods are after-treated by steaming and rinsing as described in Example 10. Grey colored slubbing is obtained which is distinguished by a full, voluminous feel. The goods can be well combed and spun.

60 65 70 75

## Example 32

13 parts of the chromium-containing monoazo dyestuff: 2 - hydroxy - 5 - methylsulfonyl - 1 - aminobenzene  $\rightarrow$  1 - acetyl amino-7-hydroxynaphthalene are pasted with 60 parts of cold water and then completely dissolved in 890 parts of hot water with heating to 80° (dyestuff:chromium=2:1). To the hot solution there is added while stirring a mixture of 10 parts of locust bean flour and 3 parts of ethanol, and after cooling to 50°, 20 parts of a mixture prepared from 10 parts of coconut oil fatty acid N-methyl-N-( $\beta$ -hydroxyethyl)-amide, 10 parts of sodium p-dodecyl-benzene-sulfonate and 2 parts of isopropanol. To the solution thus obtained there are added 10 parts of 80%-acetic acid and 10 parts of water. The temperature of the solution should be about 50°.

Wool slubbing is impregnated with this liquor at 50°, the goods are squeezed out to leave a liquid content of about 105% calculated on their dry weight, and then steamed at 100-102° with saturated steam under slight excess pressure for 15 minutes. The fabric is then rinsed first with 40° warm water then with an aqueous solution of nonylphenol heptaglycol ether at 40°, and finally rinsed with cold water and dried.

A very level grey wool slubbing of good penetration is obtained. It shows no sandwich effect.

If the steaming time in the above example is increased to 30 or 60 minutes, then dyeings of increasingly greater color strength but otherwise of the same value are obtained.

Dyeings of similar quality are also obtained when using in lieu of the 30 g. of dye assistant mixture mentioned above, one of the mixtures (a) to (t) of Example 22.

## Example 33

16 parts of the dyestuff sulfanilic acid  $\rightarrow$  1-hydroxy-[3' - trichloropyrimidylamino] - benzoylaminonaphthalene-3,6-disulfonic acid are stirred into a paste with 40 parts of water and then dissolved by the addition of 890 parts of hot water with heating. 10 parts of carob bean flour which has been previously made into a paste with a small amount of ethanol to improve its solubility, are added while stirring. After the thickener has dissolved, the solution is cooled to 50° and then 30 parts of a dyestuff carrier mixture consisting of 15 parts of pelargonic acid-N,N- $\beta$ -hydroxyethylamide, 15 parts of sodium 1-(1,3,5-tetramethyl-octyl)-benzene-4-sulfonate and 2 parts of isopropanol as well as 10 parts of 85%-formic acid and 30 parts of water are added thereto.

Wool slubbing is impregnated with this padding liquor at 50° and then squeezed out on a padding mangle to a squeezing effect of about 100% increase in weight. The slubbing is subsequently steamed for 15 minutes in saturated steam at 100-102°. After the steaming it is rinsed with warm water of about 40° and then washed at 40° with an aqueous solution containing 1 g./liter of nonylphenolpolyglycol ether, then rinsed and dried. A red dyed slubbing without sandwich effect is obtained.

If 5 parts of sodium copperphthalocyanine-disulfonate are used instead of 16 parts of the above mentioned azo dyestuff and otherwise the procedure given in the example is followed, then a turquoise-blue dyed slubbing of similar good quality is obtained.

If one of the mixtures (a) to (j) of Example 22 is used instead of the dyestuff carrier mixture given in the above example and otherwise the procedure given in the example is followed, then a red or turquoise-blue dyed slubbing without sandwich effect is obtained.

## Example 34

80 parts of Eriochrome Black T (Mordant Black 11) and 5 parts by volume of 25% aqueous ammonia are dissolved in hot water and this solution is treated with 100

parts by volume of a 2.5% glactomann solution and 30 parts of a mixture of:

15 parts of coconut oil fatty acid-N,N-bis-( $\beta$ -hydroxyethyl)-amide and

5 15 parts of sodium p-(n-dodecylbenzene)-sulfonate in 500 parts by volume of warm water.

A mixture consisting of:

20 parts of sodium fluoride and

10 50 parts by volume of aqueous 20% chromium acetate solution,

which mixture has been previously brought to the boil, is added to the solution and the whole is then made up to 900 parts by volume with warm water. 20 parts by volume of aqueous 85% formic acid are added to the solution. The solution is then brought up to 1000 parts by volume by adding water. The temperature of the finished solution should be about 50°.

Wool slubbing is impregnated at 50° with this dyebath, squeezed out to a liquor content of about 100% and steamed with saturated steam at 98° for 30 minutes.

Hereafter the slubbing is rinsed out at 40° in a first bath in a back-washing machine and treated for 15 to 30 seconds at a temperature of 70° in a second back-washing bath with a solution of:

10 g./liter of sodiumbichromate and  
8 ml./liter of 85% formic acid.

The slubbing is then rinsed out in the further back-washings with water of about 40°.

A levelly dyed black wool slubbing is obtained which is easily combed and spun.

## Example 35

35 If, instead of the 2:1 chromium complex dyestuff of Example 24, 50 parts of the dyestuff mixture consisting of the orange colored 2:1 chromium complex dyestuff of the formula



50 the red dyestuff of the formula



65 and the blue dyestuff of the formula



## 25

(weight ratio 22:22:6) and 15 instead of 20 parts by volume of 85% formic acid are used and otherwise the procedure given in Example 24 is followed, then levelly dyed brown-red wool slubbing with similar properties is obtained.

## Example 36

A fabric consisting of 45 parts of wool and 55 parts of polyethylene glycol terephthalate fibers is impregnated and steamed analogously to Example 24. The woolen portion of the fabric is dyed orange, while the polyester portion remains practically undyed.

## Example 37

A mixed fabric of wool and cellulose triacetate is impregnated and steamed analogously to Example 24. The woolen portion of the fabric is dyed orange, while the triacetate portion remains practically undyed.

## Example 38

## 11 parts of the dyestuff of the formula



are dispersed in an 80° warm mixture of 200 parts of a 35 2.5% aqueous sodium alginate solution and 35 parts of a dyestuff carrier mixture consisting of: 20 parts of coconut fatty acid-N,N-di-β-hydroxy-ethylamide, 15 parts of sodium p-decylphenolsulfonate and 2 parts of isopropanol. The solution obtained is made up with warm water to 40 about 1000 parts, whereby the pH should be about 7.

Orlon-type polyacrylonitrile slubbing (containing per 100 grams of fibers 46 millimols of sulfo groups and 17 millimols of carboxyl groups) is impregnated at 30° with this solution, squeezed out to about 100% (calculated on the dry weight) and steamed at 98° for 30 minutes with saturated steam. It is then washed out with an aqueous solution containing 1 g./liter of nonylphenol-polyglycol ether and rinsed with cold and warm water. A yellow dyed slubbing is obtained.

If, instead of the 10 parts of the given dyestuff, the same amount of 1 - amino - 2 - methoxy-4-hydroxy-anthraquinone dyestuff is used and otherwise the procedure given in the example is followed, then red dyed orlon slubbing is obtained.

Instead of the above-mentioned orlon-type fibers, Acrlan-type acrylic fibers which are copolymers from 85% acrylonitrile and 15% vinyl acetate, can be dyed successfully with the same padding liquors and in the same manner as described in Example 38.

## Example 39

Polyethyleneglycol terephthalate slubbing is impregnated at 30° with a padding liquor prepared according to Example 29 and squeezed out to a liquor content of 80%.

The slubbing is steamed at 98° for 30 minutes with saturated steam, washed subsequently with an aqueous solution containing 1 g./liter of nonylphenol-polyglycol ether and rinsed out with warm and cold water. A levelly dyed 70 yellow or red polyester slubbing is obtained.

If 5 parts of o-phenylphenol is added to the above padding liquor and the same procedure as given in the example is followed, then a yellow or red dyed slubbing of stronger color is obtained.

## 26

## Example 40

20 parts of the dyestuff of the formula



are dissolved in a 60° warm mixture of 200 parts by volume of a 2.5% aqueous solution of "Meyprogum KN" and 30 parts of a dyestuff carrier consisting of:

15 9 parts of sodium 4-(1-methyl-undecyl)-benzene-1-sulfonate,

9 parts of coconut fatty acid-N,N-bis-(β-hydroxyethyl) amide and

250 parts by volume of water.

20 The solution obtained is diluted with warm water to about 900 parts by volume and the pH value of the solution is adjusted to 4 with 80% acetic acid.

Orlon-type slubbing of the same kind as used in Example 38 is impregnated at 30° with this solution, squeezed out to about 130% (calculated on the dry weight) and steamed at 98° for 30 minutes with saturated steam. It is then washed with a solution containing 1 g./liter of

25 nonylphenol-polyglycol ether and rinsed with warm and cold water. A yellow dyed acrylic slubbing is obtained.

30 If, instead of the dyestuff given above, the dyestuff Maxilon Red BL (C.I. Basic Red 22) is used and the procedure given in the example is followed, then red dyed acrylic slubbing of similar good quality is obtained.

Instead of the above orlon-type fibers, Acrlan type acrylic fibers as used in Example 38 can be dyed with the same padding liquors and in the same manner as described in Example 40, supra, and similar satisfactory results are obtained.

## Example 41

35 360 parts of the dyestuff 1-amino-6-nitro-2-hydroxy-naphthalene-4-sulfonic acid→2-hydroxynaphthalene in the form of a press cake are added, while stirring, in portions to a boiler fitted with a turbo mixer already containing 360 parts of water, and stirred for one hour. In a second 45 mixing vessel 120 parts of a dyestuff carrier mixture consisting of 60 parts of coconut fatty acid-N,N-di-(β-hydroxy-alkylamide), 60 parts of sodium 4-(1-methyl-undecyl)-benzene-sulfonate and 10 parts of 80% acetic acid are mixed. This homogeneous mixture is poured slowly, while stirring, into the dyestuff suspension and the whole is subsequently stirred for 15 minutes more, whereby a 50 homogeneous, brown, ready-for-use dye composition is obtained.

55 A pad liquor is prepared from this composition by mixing 300 parts of the same with 350 parts of warm water of 60° and 100 parts of an aqueous 2.5% solution of carob bean flour thickener. 40 parts of chromium trifluoride and 20 parts of 85% formic acid are added to the resulting solution and the dyebath is made up to 1000 parts by volume with warm water. Wool slubbing is then 60 impregnated with this dyebath as described in Example 22.

A level-dyed black-colored wool slubbing is obtained that is easily combed and spun. The dyeing has good wash and light fastness and is free from sandwich effect.

65 By following the procedure outlined in the first paragraph of Example 41, supra, and using press cakes of the other dyestuffs used in the preceding examples, other well storables ready-for-use compositions are obtained, from which pad liquors can be easily prepared by the procedure described in the second paragraph of Example 41.

We claim:

1. In a process for the dyeing of polyamide fibers by 75 impregnating them with a thicker-than-water aqueous solu-

tion of an acid wool dyestuff at a temperature below the drawing temperature for the dyestuff and then heating the impregnated goods in a humid medium, the improvement which comprises:

(a) adding to the said aqueous solution, prior to the impregnation of the fibers therewith,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

2. In a process for the dyeing of polyamide fibers by impregnating them by a method of printing with a thicker-than-water aqueous solution of an acid wool dyestuff at a temperature below the drawing temperature for the dyestuff and then heating the printed goods in a humid medium, the improvement which comprises:

(a) adding to the said aqueous solution, prior to the printing of the fibers therewith,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acids and thioglycolic acid, and a mixture of  $\alpha$ - and  $\beta$ -tetrahydronaphthalene sulfonic acids and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

3. In a process for the dyeing of polyamide fibers by impregnating them by a method of coating with a thicker-than-water aqueous solution of an acid wool dyestuff at a temperature below the drawing temperature for the dyestuff and then heating the coated goods in a humid medium, the improvement which comprises:

(a) adding to the said aqueous solution, prior to the coating of the fibers therewith,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids and thioglycolic acid, and

75

acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral alkaline value, the simultaneous presence of auxiliaries (1) and (2) preventing separation of said impregnation liquor into two phases, one of which is poor and the other rich in the said auxiliaries.

4. In a process for the dyeing of polyamide fibers by impregnating them by a method of spraying with a thicker-than-water aqueous solution of an acid wool dyestuff at a temperature below the drawing temperature for the dyestuff and then heating the spray-impregnated goods in a humid medium the improvement which comprises:

(a) adding to the said aqueous solution, prior to the impregnation of the fibers therewith,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

5. In a process for the dyeing of polyamide fibers by impregnating them by a method of pad dyeing with a thicker-than-water aqueous solution of an acid wool dyestuff at a temperature below the drawing temperature for the dyestuff and then heating the impregnated goods in a humid medium, the improvement which comprises:

(a) adding to the said aqueous solution, prior to the foulard-impregnation of the fibers therewith,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

6. In a process for the dyeing of polyamide fibers by impregnating them by a method of printing with a thicker-than-water aqueous solution of an acid wool dyestuff at a temperature below the drawing temperature for the dyestuff and then steaming the impregnated goods in a humid medium, the improvement which comprises:

(a) adding to the said aqueous solution prior to the printing of the fibers therewith,

(1) as color transfer agent, a water-soluble con-

- densation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acids, a mixture of  $\beta$ -tetrahydronaphthalene sulfonic acid and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
7. In a process for the dyeing of polyamide fibers by impregnating them by a method of coating with a thicker-than-water aqueous solution of an acid wool dyestuff at a temperature below the drawing temperature for the dyestuff and then steaming the impregnated goods in a humid medium, the improvement which comprises:
- (a) adding to the said aqueous solution, prior to the coating of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
8. In a process for the dyeing of polyamide fibers by impregnating them by a method of spraying with a thicker-than-water aqueous solution of an acid wool dyestuff at a temperature below the drawing temperature for the dyestuff and then steaming the impregnated goods in a humid medium, the improvement which comprises:
- (a) adding to the said aqueous solution, prior to the spray-impregnation of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acid, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

9. In a process for the dyeing of polyamide fibers by impregnating them by a method of pad-dyeing with a thicker-than-water aqueous solution of an acid wool dyestuff at a temperature below the drawing temperature for the dyestuff and then steaming the impregnated goods in a humid medium, the improvement which comprises:
- (a) adding to the said aqueous solution, prior to the foularding of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
10. In a process for the dyeing of polyamide fibers by impregnating them by a method of printing with a thicker-than-water aqueous solution of an acid wool dyestuff at a temperature below the drawing temperature for the dyestuff and then passing the impregnated goods through a hot acid shock bath, the improvement which comprises:
- (a) adding to the said aqueous solution, prior to the printing of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
11. In a process for the dyeing of polyamide fibers by impregnating them by a method of coating with a thicker-than-water aqueous solution of an acid wool dyestuff at a temperature below the drawing temperature for the dyestuff and then passing the impregnated goods through a hot acid shock bath, the improvement which comprises:
- (a) adding to the said aqueous solution, prior to the coating of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

- acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
12. In a process for the dyeing of polyamide fibers by impregnating them by a method of spraying with a thicker-than-water aqueous solution of an acid wool dye-stuff at a temperature below the drawing temperature for the dyestuff and then passing the impregnated goods through a hot acid shock bath, the improvement which comprises:
- (a) adding to the said aqueous solution, prior to the spray-impregnation of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
13. In a process for the dyeing of polyamide fibers by impregnating them by a method of pad-dyeing with a thicker-than-water aqueous solution of an acid wool dye-stuff at a temperature below the drawing temperature for the dyestuff and then passing the impregnated goods through a hot acid shock bath, the improvement which comprises:
- (a) adding to the said aqueous solution, prior to the fouldering of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
14. In a process for the dyeing of polyamide fibers by impregnating them by a method of printing with a thicker-than-water aqueous solution of an acid wool dye-stuff at a temperature below the drawing temperature for the dyestuff and subsequently steaming the impregnated goods in a humid medium and then passing the steamed goods through a hot acid shock bath, the improvement which comprises:

- (a) adding to the said aqueous solution, prior to the printing of the fibers therewith
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
15. In a process for the dyeing of polyamide fibers by impregnating them by a method of coating with a thicker-than-water aqueous solution of an acid wool dye-stuff at a temperature below the drawing temperature for the dyestuff and subsequently steaming the impregnated goods in a humid medium and then passing the steamed goods through a hot acid shock bath, the improvement which comprises:
- (a) adding to the said aqueous solution, prior to the coating of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.
16. In a process for the dyeing of polyamide fibers by impregnating them by a method of spraying with a thicker-than-water aqueous solution of an acid wool dye-stuff at a temperature below the drawing temperature for the dyestuff and subsequently steaming the impregnated goods in a humid medium and then passing the steamed good through a hot acid shock bath, the improvement which comprises:
- (a) adding to the said aqueous solution, prior to the spray-impregnation of the fibers therewith,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

17. In a process for the dyeing of polyamide fibers by impregnating them by a method of foularding with a thicker-than-water aqueous solution of an acid wool dyestuff at a temperature below the drawing temperature for the dyestuff and subsequently steaming the impregnated goods in a humid medium and then passing the steamed goods through a hot acid shock bath, the improvement which comprises:

(a) adding to the said aqueous solution, prior to the foularding of the fibers therewith,

- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries.

18. In a process for the dyeing of polyamide fibers by applying to them a thicker-than-water aqueous solution of an acid wool dyestuff at a temperature below the drawing temperature for the dyestuff and heating the impregnated goods in a humid medium, the improvement which comprises:

(a) adding to the said aqueous solution,

- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

(b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries,

(c) applying said liquor to said fibers, and

(d) subsequently heating the impregnated fibers in said humid medium directly without intermediate drying.

19. In a process for the dyeing of polyamide fibers by impregnating them by a method of printing with a thicker-than-water aqueous solution of an acid wool dyestuff at a temperature below the drawing temperature for the dyestuff and heating the impregnated goods in a humid medium, the improvement which comprises:

(a) adding to the said aqueous solution,

- (1) as color transfer agent, a water-soluble condensation product of one equivalent of fatty acid having 8 to 14 carbon atoms with from

5 one to three equivalents of a member selected from the group consisting of dialkanolamine with from 4 to 6 carbon atoms and trialkanolamine with from 6 to 9 carbon atoms, and

10 (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, and

15 (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries,

(c) printing said fibers with the said liquor, and

(d) subsequently heating the printed goods in said

20 humid medium directly without intermediate drying.

25 20. In a process for the dyeing of polyamide fibers by impregnating them by a method of coating with a thicker-than-water aqueous solution of an acid wool dyestuff at a temperature below the drawing temperature for the dye-  
25 stuff and heating the impregnated goods in a humid me-  
dium, the improvement which comprises:

(a) adding to the said aqueous solution

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid,

30 (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries,

(c) coating said fibers with the resulting liquor, and

(d) subsequently heating the coated goods in said humid medium directly without intermediate drying.

35 21. In a process for the dyeing of polyamide fibers by impregnating them by a method of spraying with a thicker-than-water aqueous solution of an acid wool dyestuff at a temperature below the drawing temperature for the dyestuff and heating the impregnated goods in a humid medium, the improvement which comprises:

(a) adding to the said aqueous solution,

(1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid,

40 (b) adjusting the pH of the resultant impregnation liquor to a neutral to alkaline value, the simultaneous presence of auxiliaries (1) and (2) preventing separation of said impregnation liquor into two phases,

- one of which is poor and the other rich in the said auxiliaries,
- (c) spray-impregnating said fibers with the resulting liquor, and
- (d) subsequently heating the spray-impregnated goods in said humid medium directly without intermediate drying.

22. In a process for the dyeing of polyamide fibers by impregnating them by a method of pad-dyeing with a thicker-than-water aqueous solution of an acid wool dyestuff at a temperature below the drawing temperature for the dyestuff and heating the impregnated goods in a humid medium, the improvement which comprises:

- (a) adding to the said aqueous solution,
- (1) as color transfer agent, a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (2) a member selected from the group consisting of  $\beta$ -tetrahydronaphthalene sulfonic acid, a mixture of  $\alpha$ - and  $\beta$ -tetrahydronaphthalene sulfonic acids, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid,
- (b) adjusting the pH of the resultant impregnation liquor to a neutral to alkaline value, the simultaneous presence of auxiliaries (1) and (2) preventing separation of said impregnation liquor into two phases, one of which is poor and the other rich in the said auxiliaries,
- (c) foularding said fibers with the resulting liquor, and
- (d) subsequently heating the foularded goods in said humid medium directly without intermediate drying.

23. In a process for the dyeing of polyamide fibers by impregnating them with a thicker-than-water aqueous solution of an acid wool dyestuff at a temperature below the drawing temperature for the dyestuff and then heating the fibers in a humid medium, the improvement which comprises:

- (a) adding to the said aqueous solution, prior to the impregnation of the fibers therewith,
- (1) as color transfer agent, a water-soluble reaction product of one equivalent of fatty acid having 8 to 14 carbon atoms with from one to three equivalents of a member selected from among dialkanolamine with from 4 to 6 carbon atoms and trialkanolamine with from 6 to 9 carbon atoms, and
- (2) as anionic "steam-blowing" control agent, a substance selected from among:
- ( $\alpha$ ) a sulfonated alkyl-benzene wherein the alkyl moiety has from 8 to 20 carbon atoms,
- ( $\beta$ ) sulfonated  $\beta$ -tetrahydronaphthalene,
- ( $\beta'$ ) a mixture of sulfonated  $\alpha$ - and  $\beta$ -tetrahydronaphthalene,
- ( $\beta''$ ) a mixture of sulfonated  $\beta$ -tetrahydronaphthalene and thioglycolic acid,
- ( $\beta'''$ ) a mixture of sulfonated  $\alpha$ - and  $\beta$ -tetrahydronaphthalene and thioglycolic acid,
- ( $\gamma$ ) condensation products of formaldehyde or, glyoxal or acetaldehyde with per mole thereof, about 1.2 to 2 moles of at least one of the following compounds:
- ( $\delta$ ) a mixed disulfonated diaryl-alkane which is a condensation product of (i) naphthalene-sulfonic acid, (ii) a member selected from among benzene-sulfonic acid and p-toluene-sulfonic acid, and (iii) a member selected from among formaldehyde and a lower alkylene-dialdehyde of from 2 to 8 carbon atoms; and

(b) adjusting the pH of the resultant impregnation liquor to a value in the range of from 2 to 9, the simultaneous presence of auxiliaries (1) and (2) suppressing the formation of sandwich effects in the dyed fibers.

24. The improvement as defined in claim 23, further comprising:

- (c) applying the resulting liquor to said fibers, and
- (d) subsequently heating the fibers in said humid medium directly without intermediate drying.

25. The improvement defined in claim 24, wherein said liquor is applied to said fibers by printing.

26. The improvement defined in claim 24, wherein said liquor is applied to said fibers by padding and subsequent mechanical removal of excess liquor from the fibers.

27. The improvement defined in claim 24, wherein said liquor is applied to said fibers by coating.

28. The improvement defined in claim 24, wherein said liquor is applied to said fibers by spraying the latter therewith.

29. The improvement defined in claim 26, wherein the pH of the liquid is adjusted to a neutral to alkaline value within the range given, and which improvement further comprises:

- (e) passing the fibers obtained by step (d) through an acid shock bath.

30. An impregnation liquor for the dyeing of polyamide fibers, consisting essentially of:

- (1) a thicker-than-water aqueous solution of an acid wool dyestuff,
- (2) as color transfer agent a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and

(3) a member selected from the group consisting of  $\beta$ -tetrahydronaphthalene sulfonic acid, a mixture of  $\beta$ -tetrahydronaphthalene sulfonic acid and thioglycolic acid, and a mixture of  $\alpha$ - and  $\beta$ -tetrahydronaphthalene sulfonic acids and thioglycolic acid, the ratio of said color transfer agent to said member defined under (3) ranging from about 2.5:1 to 4:1, the simultaneous presence of auxiliaries (2) and (3) preventing separation of said impregnation liquor into two phases, one of which is poor and the other rich in the said auxiliaries.

31. An impregnation liquor as defined in claim 30, wherein the effective amount of said color transfer agent is between 10 to 60 grams per liter.

32. An impregnation liquor as defined in claim 30, wherein the member defined under (3) is present in an amount of 2 to 20 grams per liter.

33. An impregnation liquor as defined in claim 30, wherein the member defined under (3) is  $\beta$ -tetrahydronaphthalene sulfonic acid.

34. An impregnation liquor as defined in claim 30, wherein the member defined under (3) is a mixture of  $\beta$ -tetrahydronaphthalene sulfonic acid and thioglycolic acid, the latter being present in an amount from 0.1 to 3 grams per liter of said liquor.

35. An impregnation liquor as defined in claim 30, wherein the member defined under (3) is a mixture of  $\alpha$ - and  $\beta$ -tetrahydronaphthalene sulfonic acids and thioglycolic acid, the latter being present in an amount from 0.1 to 3 grams per liter of said liquor.

36. An impregnation liquor as defined in claim 30, wherein the color transfer agent is a water-soluble condensation product of one equivalent of coconut fatty acid with two equivalents of diethanolamine.

37. An impregnation liquor for the dyeing of polyamide fibers, consisting essentially of:

- (1) a thicker-than-water aqueous solution of an acid wool dyestuff,

- (2) as color transfer agent a water-soluble condensation product of one equivalent of fatty acid having 8 to 14 carbon atoms with from one to three equivalents of a member selected from the group consisting of dialkanolamine with from 4 to 6 carbon atoms and trialkanolamine with from 6 to 9 carbon atoms, and
- (3) as anionic "steam-blowing" control agent, a substance selected from among:
- (α) a sulfonated alkyl-benzene wherein the alkyl moiety has from 8 to 20 carbon atoms,
  - (β) sulfonated  $\beta$ -tetrahydronaphthalene,
  - (β') a mixture of sulfonated  $\alpha$ - and  $\beta$ -tetrahydronaphthalene,
  - (β'') a mixture of sulfonated  $\beta$ -tetrahydronaphthalene and thioglycolic acid,
  - (β''') a mixture of sulfonated  $\alpha$ - and  $\beta$ -tetrahydronaphthalene and thioglycolic acid,
  - (γ) condensation products of formaldehyde, or glyoxal, or acetaldehyde with, per mole thereof, about 1.2 to 2 moles of at least one of the following compounds:
    - (i) benzene-sulfonic acid,
    - (ii) naphthalene-sulfonic acid,
    - (iii) tetrahydronaphthalene-sulfonic acid,
    - (iv) a methyl-substituted compound of (i) to (iii) inclusive, in free acid form or in the form of water-soluble salts thereof; the ratio of said color transfer agent to said member defined under (3) ranging from about 5:1 to 1:3.

38. An impregnation liquor as defined in claim 37, wherein the effective amount of said color transfer agent is between 10 to 60 grams per liter.

39. An impregnation liquor as defined in claim 37, wherein the agent defined under (3) is present in an amount of 2 to 20 grams per liter.

40. An impregnation liquor as defined in claim 37, wherein the member defined under (3) is  $\beta$ -tetrahydronaphthalene sulfonic acid.

41. An impregnation liquor as defined in claim 37, wherein the member defined under (3) is a mixture of  $\beta$ -tetrahydronaphthalene sulfonic acid and thioglycolic acid, the latter being present in an amount from 0.1 to 3 grams per liter of said liquor.

- 5 42. An impregnation liquor as defined in claim 37, wherein the member defined under (3) is a mixture of  $\alpha$ - and  $\beta$ -tetrahydronaphthalene sulfonic acids and thioglycolic acid, the latter being present in an amount from 0.1 to 3 grams per liter of said liquor.
- 10 43. An impregnation liquor as defined in claim 37, wherein the color transfer agent is a water-soluble condensation product of one equivalent of coconut fatty acid with two equivalents of diethanolamine.
- 15 44. An impregnation liquor as defined in claim 37, wherein the member defined under (3) is a sulfonated alkyl-benzene wherein the alkyl moiety has from 8 to 20 carbon atoms.
- 20 45. An impregnation liquor as defined in claim 37, wherein the member defined under (3) is a mono-sulfonated-dodecylbenzene.
- 25 46. An impregnation liquor as defined in claim 37, wherein the member defined under (3) is monosulfonated p-(1,3,3,5-tetramethyl-octyl)-benzene.
- 30 47. An impregnation liquor as defined in claim 37, wherein the member defined under (3) is disulfonated dinaphthyl-alkane, wherein the alkane moiety has from 1 to 2 carbon atoms, and the two naphthyl radicals are each linked to a different carbon atom thereof.
- 35 48. An impregnation liquor as defined in claim 37, wherein the member defined under (3) is disulfonated naphthyl-methane.
- 40 49. An impregnation liquor as defined in claim 37, wherein the ratio of said color transfer agent to said member defined under (3) is about 3:1.

#### References Cited

##### UNITED STATES PATENTS

|           |        |           |       |        |
|-----------|--------|-----------|-------|--------|
| 1,926,556 | 9/1933 | Nuesslein | ----- | 8—89 X |
| 2,552,404 | 5/1951 | Casty     | ----- | 8—54 X |
| 2,828,180 | 3/1958 | Sertorio  | ----- | 8—93 X |

40 NORMAN G. TORCHIN, Primary Examiner

T. J. HERBERT, Jr., Assistant Examiner

U.S. Cl. X.R.

45 8—55, 85, 89